

## UNITED STATES PATENT OFFICE

2,611,678

## TRANSPARENTIZING TO OBTAIN PATTERNED COTTON TEXTILES EMPLOYING RESISTS OF PIGMENT CONTAINING AQUEOUS OLEAGINOUS EMULSIONS

Heinz Ginzel, Dornbirn, Vorarlberg, Austria

No Drawing. Application July 11, 1947, Serial No. 760,513. In Germany October 18, 1941.

Section 1, Public Law 690, August 8, 1946  
Patent expires October 18, 1961

7 Claims. (Cl. 8—115)

1

This invention relates to improvements in or relating to figured textiles.

For obtaining figured effects on fabrics by printing with pigments, the pigments are fixed on the surface of the fabrics by the aid of binding materials. Albumines (e. g. albumine, caseine, coagulated or hardened gelatine), natural and artificial resins, and derivatives of cellulose have been used as binding materials. These binding substances however are not removable by washing. The same binding materials are used, when fabrics, printed with pigments, are treated, before and/or after the printing, once or several times with lye and/or acids or other hydrolysing agents to improve the same and especially to impart thereto a transparent appearance. Thus it is known, that completely stiffened figured effects on loose, broad looped textile surfaces are obtained by printing them with a solution containing pigment and/or cellulose or instead of the cellulose, albumine or resins and to parchmentise the fabric after the fixation of the resist layer produced by the printing. Particularly the use of carbamide-formaldehyde condensates, as dimethylolcarbamide and melamine-formaldehyde-condensates, phenol-formaldehyde-condensates and polymerisates, e. g. polystyrol as binding materials has been utilized for obtaining figured effects by pigment printing in combination with a subsequent parchmentizing process. With such a process, the eventual addition of plasticizing agents to condensates of an aminoderivative of triazine with an aldehyde, has been suggested and olive oil, glycerine, paraffine oil, and certain quaternary ammonium compounds were mentioned as examples. The addition of hydrophobe compounds as paraffin, wax, resins and aluminum salts to such binding compounds has been considered but the binding of the pigments has been obtained in such compositions by the use of artificial resins, the hardness and stiffness of which has been reduced by such additions.

This invention aims at providing cellulosic textile goods for instance cotton fabrics, such as organdie, in which certain defined areas are of permanent transparency and other defined areas are non transparent, the non transparent areas being pigmented without imparting to the textile goods an additional stiffening at the non-transparent parts. Another object of this invention is to provide such textile goods having a clear pattern of great lucidity and beauty and in which each

2

thread is visible within the pigmented area. Another object of the invention is to provide a process for producing textile goods having the qualities mentioned above. Other objects of the invention will appear as the description proceeds.

According to the invention figured cellulosic textiles are provided which comprise defined areas of permanent transparency and defined areas of a nontransparent character, the fibres within the latter areas being pigmented with the aid of a hydrophobic substance of a fatty character containing coloring pigments. By the terms hydrophobic substance of a fatty character I include such substances which have the physical qualities of fats, that is to say oleaginous substances which exercise a repellent action against water and aqueous solutions, but are capable of being emulsified, and which are capable of forming smooth and non-cracking deposits or films on a base on which they are applied. Examples of such substances of fatty character are higher hydrocarbons, particularly paraffin, glycerides, for example animal or vegetable oils and fats, waxes and higher fatty acids, commonly occurring in natural fats and oils or mixtures thereof.

For producing figured textiles for instance woven or knitted fabrics or yarns, especially from native cellulose, according to the invention the fabrics are printed in pattern with printing pastes, which contain pigments and/or compounds which form pigments by hydrolysis or thermal decomposition, and besides auxiliary printing agents removable by washing, and oleaginous substances such as hydrocarbons, glycerides, waxes, higher fatty acids or their salts or a mixture of these substances in the form of an emulsion, these substances being per se hydrophobic or forming hydrophobic substances when treated by concentrated acids. The printed textiles are then dried and/or steamed and treated with concentrated acid, preferably sulphuric acid of more than 40° Bé, or agents reacting in the same way for obtaining a permanent fixation of the pigments.

Printing pastes comprising emulsions of paraffin or cerine or beeswax, or of tallow, stearine, stearine soaps or wax soaps, to which have been added emulgents, protective colloids, or other additional and auxiliary compounds may be used according to the invention. Such oleaginous substances may also be made emulsive in water by sulphonation or partial sulphonation. If salts of fatty acids (soaps) are used as the fatty com-

ponent of the printing paste, the insoluble hydrophobe fatty acids are precipitated on the fibre by the subsequent treatment with concentrated acids.

Metal-salts, such as aluminum salts which electrically charge or reverse the electric charge of the emulsions to the positive may be incorporated in the printing pastes or in the emulsions of the fatty substance used for preparing the printing pastes. Such emulsions have heretofore been used in the form of diluted baths for the porous-hydrophobe impregnation of textiles while they are used according to the invention as printing pastes for obtaining local patterns.

Prefabricated pigments may be added to the printing pastes used according to the invention or, the same result may be accomplished by utilizing metal salts, which by hydrolysis or thermal decomposition under the conditions of the process form insoluble precipitates which serve as the pigment substance. Such salts may also be used, which at the same time electrically charge or reverse the electrical charge of the emulsion to the positive.

Surprisingly, it has been proved, that the emulsions, which are frequently not completely coagulated, when brought on the fibre and subsequently dried and eventually steamed, coagulate completely at a subsequent treatment with acid, for instance concentrated sulphuric acid of more than approximately 40° Bé., preferably 45° to 55° Bé., as used for producing translucent effects transparentising and parchmentising or producing linen-like effects, or with other similarly acting swelling agents. By this, the insoluble compounds of the printing paste are very stably fixed on and in the fibre. Upon this treatment with acid, a very strong bonding between the hydrophobic precipitate and the fibre is established. This binding action may result from electrical reverses and discharges between the fibre, the emulsion colloids or the product of the coagulation, the metal salt and the concentrated acid. As a result, a part of the pigments added to the printing paste is surrounded by the precipitated compounds and fixed on the fibre in a manner which is surprisingly resistant against rubbing, washing and boiling. The unbound surplus of the pigments is preferably removed by washing before the textiles are treated on frames and finished. The treatment of the printed fabrics with acids is effected without shrinking by employing simultaneous or subsequent tension, thereby producing a surface pattern on the fabric.

Examples of various prefabricated pigments, which may be incorporated into the printing paste are: titanium dioxide, zinc white, permanent white, kaolin, lithopone, colloidal silicic acid, and other equivalent mineral pigment substances.

Instead of the prefabricated pigments, or in addition thereto, solutions of metal salts may be added to the printing paste which yield pigments as a result of the drying or steaming step by a hydrolysis or thermal decomposition, leading to a precipitation of white, insoluble oxides on the fibre which make the fibre dull and which are resistant against washing. Solutions of basic salts of similar qualities may also be used. For this purpose, preferably non-corroding aluminium-, antimony-, bismuth-, tin-, lead-, zinc, and magnesium salts, as aluminium acetate, aluminium formiate, aluminium-salts of aromatic orthodicarboxic acids or their derivatives, as phthalic acid, tetrachloric phthalic acid, antimony-potas-

sium-tartrate, lead chloride, bismuth carbonate, stannates of alkalin, zinc acetate, or magnesium chloride are used. The precipitates, originated from these metal salt solutions during the treatment are resistant against washing and boiling.

It is useful to add cation active compounds to the printing paste, like lauryl pyridinium sulphate, which are able to charge or to recharge the pastes electrically, or to use a pigment suspension, obtained from such cation active compounds, in the printing paste. To adjust the printing qualities of the printing paste, additional and auxiliary compounds conventionally used in cloth printing and which are removable by washing are added, singly or in a mixture, as diluting, thickening, plastifying, softening or stiffening agents or agglutinants. Also filling, lustre making, dull making, metallising, corroding, luminescent or dyeing compounds may be added to the printing paste.

It is remarkable, that usually only a comparatively small percentage of hydrophobic emulsified compounds in the printing paste is sufficient to produce the results aimed at by the invention, as will be apparent from the herein-after described processes and examples which set forth representative compositions of a printing paste formulated according to the invention.

The process according to the invention may be used for obtaining patterns on cotton textiles. The textiles to be subjected to the process according to the invention may be in a raw state or partially refined, e. g. bleached, mercerised, dyed, calendered or in any other way pretreated or retreated, either as to a part of the yarns or completely. The textiles may be of various density and weave and may contain yarns of equal or unequal quality or strength and twisting or overtwisting.

This process may also be combined with one of the known refining processes, as for instance an impregnation or an antirumpling treatment, for instance with artificial resins such as dimethylcarbamide, or a finishing process, for instance with cellulose ethers. It may also be combined with an esterification or alkoxylation or with the usual pigment printing or color printing and/or local transparentizing printing, as well as with effects of embroidery, annealing, perforation, corrosion and the like. The textiles may also be dyed before or after the production of the pattern process.

All variations of printing effects, which may be realized according to the process of the invention may be produced by one or more stages either singly or in parallel, either partly or completely covering each other, with or without white and/or colored effects, with or without a local or complete swelling process.

An important way of realizing the process according to the invention, is to combine it with swelling processes of various kinds, wherein the local printing with the printing paste according to the invention may be effected before, or between two or more, or after the swelling processes. However, it is necessary in any case to fix the pigments after the printing and the subsequent steaming or drying by the treatment with concentrated sulphuric acid or similar agents. Thus the fabrics may be mercerized before the printing, or the printed fabrics may be mercerized after the treatment with acids, or they may be subjected to both treatments. By the swelling processes various effects, for instance wool like

effects, linen- or silk-like effects or opalescent, parchmentized, or transparent or similar effects may be obtained, as are well known, by different working conditions (type and concentration, temperature, time of reaction of the swelling agent, 5 addition of preservative compounds to the swelling agent, stretching of the fibre and the surface during the treatment, local reaction or reaction on the whole surface, direct printing or reserve printing, combined with a swelling process on 10 the whole surface, producing a single or parallel or partly or completely covering pattern).

The products obtained by the process according to the invention show a very considerable difference compared to the known figured fabrics, the 15 advantages being particularly apparent when employed in connection with loose fabrics having broad loops, since the manner of the local covering of the threads with this process is essentially different than that accomplished by any heretofore known. With the process according to the invention only the single threads in the parts 20 printed with the pattern are covered, while the spaces between the threads are not filled. The same effect is secured in the printed parts of a cotton muslin fabric for instance, each thread 25 remaining visible, while the unfixed printing paste between the threads is removed by washing. After passing the printed fabric through a bath of sulphuric acid or other transparentizing agent 30 the comparatively small amount of insoluble hydrophobic compounds is precipitated on and in the fibre, which after the removal of the surplus of emulsion and pigments forms a pattern of great lucidity and beauty and which possesses a 35 great resistance against soap, boiling, rubbing and light. The prints produced in accordance with the invention do not tend to dust off, as happens frequently when the usual pigment binding agents are used and which in the case of patterns 40 with a large surface, cover or fill a part of the space between the threads of the fabric. The textiles figured by the process according to the invention also show an outstanding equality and 45 homogeneity of the print. The parts figured with pigments also have a softer quality than the transparent parts and a flexible touch, which appears advantageously with pigment patterns on certain products, as handkerchiefs, curtains and linenware. The products produced by the subject invention compare favorably with products obtained by the much more difficult direct printing process with transparentizing agents. The 50 resistance of the patterns against light also offers an important advantage. The products can also be dry cleaned, since the pigments are also in this case solidly fixed on and in the fibre.

A notable feature of the invention is that the suggested printing paste may be used on the textile fibres, without damaging or weakening of the fibre by the printing.

The process according to the invention can be carried out in a simple way since emulsions of insoluble hydrophobic compounds in water are common products in commerce for the porous hydrophobic impregnation of textiles and may be utilized in preparing the described printing pastes.

#### Examples

(1) A cotton muslin, bleached and mercerized with alkali in the usual way is printed in accordance with a pattern with a printing paste of the following composition:

400 g. thickening agent: wheat starch, tragacanth 6%, water in a relation 1:2:5.  
100 g. of an aqueous emulsion of paraffin  
80 g. filtered water-glass 38° Bé. (colloidal silicate)  
200 g. titanium dioxyde 1:1  
50 g. glycerine  
160 g. water  
10 cm.<sup>3</sup> indanthrene blue 2% (Schulz Farbstofftabellen, 2 supplement 1939, page 199, Indanthrenblau R. Z.)

1000 g.

The printed fabric is then dried, steamed wet, parchmentised under tension in concentrated sulphuric acid of 54° Bé. at a temperature of 2° C. for 8 to 13 seconds, then neutralised or washed, then treated with sodium lye of 27° Bé. for 20 seconds, neutralised again and rinsed. By a subsequent frequent washing, which may be continued up to the temperature of boiling water, the surplus of pigments is removed and after a test showing the absence of pigments in the rinsing water, the fabric is eventually dressed, then treated on frames and finished. White, dull contrast patterns on a transparent ground are obtained.

(2) After the same preliminary treatment, a cotton fabric is printed with:

400 g. thickening agent: wheat starch, tragacanth 6%, water in a relation of 1:2:5  
100 g. of an aqueous emulsion of weakly sulphonated tallow  
200 g. titanium dioxyde 1:1  
50 g. glycerine  
240 cm.<sup>3</sup> water  
10 cm.<sup>3</sup> indanthrene blue 2% (Schulz Farbstofftabellen, 2 supplement 1939, page 199, Indanthrenblau R. Z.)

1000 g.

Instead of 100 g. of said aqueous emulsion of tallow, 100 g. of an emulsion of any hydrophobic substance previously specified compounds with zirconium oxychloride or zirconium oxynitrate or hydrolysates of these salts may also be used. The subsequent treatment is the same as in Example 1. White dull printing effects on a transparent ground are obtained. If a fabric dyed with indanthrene or indigosole colors is printed with this printing paste and then treated in the indicated way, white contrasts, resistant against light and washing, on a transparent colored ground are obtained.

(3) After the same preliminary treatment, a cotton muslin fabric is printed with:

450 g. thickening agent: wheat starch, tragacanth 6%, water in a relation of 1:2:5  
140 g. an aqueous emulsion of paraffin containing soluble aluminium salts  
50 g. aluminium acetate 8° Bé.  
200 g. titanium dioxyde 1:1  
50 g. glycerine  
10 g. indanthrene blue 2% (Schulz Farbstofftabellen, 2 supplement 1939, page 199, Indanthrenblau R. Z.)

70 100 cm.<sup>3</sup> water

1000 g.

This product is dried, steamed wet at a temperature of more than 100° C. and then treated

the same way as in Example 1. One obtains white, contrasting reserve patterns on a transparent ground. If the transparent product which is printed with white effects is dyed with substantive dyes, as sirius light blue, the result is effects of one tinge passing into the other.

(4) A cotton muslin fabric, bleached and mercerised in the usual way is printed with the following paste:

## I.

550 g. thickening agent: wheat starch, tragacanth 6%, water in a relation of 1:2:5  
 200 g. titanium dioxyde 1:1  
 85 g. of an aqueous emulsion of paraffin containing soluble aluminium salts  
 35 g. weakly sulfonated tallow  
 50 g. glycerine  
 75 g. water  
 10 g. indanthrene blue (Schulz Farbstofftabellen, 2 supplement 1939, page 199, Indanthrenblau R. Z.) 2%

This paste is added to the following composition:

## II.

38 g. thickening agent: wheat starch, tragacanth 6%, British gum, water, in a relation of 1:3:5  
 37 g. water  
 75 g. Indanthrene blue (Schulz Farbstofftabellen, 2 supplement 1939, page 199, Indanthrenblau R. Z.)  
 35 g. wheat starch  
 45 g. water  
 75 g. tragacanth 6%  
 15 g. British gum solid  
 45 g. glycerine  
 60 g. potassium carbonate  
 40 g. rongalite (NaHSO<sub>2</sub>.CH<sub>2</sub>O.2H<sub>2</sub>O)  
 10 g. turpentine oil  
 25 g. water

1500 g.

After the printing process, the textiles are dried and steamed in the rapid-steaming apparatus and transparentised and subsequently treated in the usual way. The result is a shining blue contrast print on a transparent ground. The composition I may also be used for obtaining white prints.

(5) A cotton muslin is bleached, mercerised and dyed light blue with a substantive dye, which may be discharged in neutral solution and then printed with:

350 g. thickening agent: wheat starch, tragacanth 6% water, in a relation of 1:2:5  
 180 g. rongalite (NaHSO<sub>2</sub>.CH<sub>2</sub>O.2H<sub>2</sub>O)  
 60 g. leucotrope (disulphonated dimethyl-phenyl-benzyl-ammonium chloride)  
 100 g. titanium dioxyde 1:1  
 100 g. zinc oxyde 1:1  
 69 g. water  
 6 g. indanthrene blue 2% (Schulz Farbstofftabellen, 2 supplement 1939, page 199, Indanthrenblau R. Z.)  
 85 g. of an aqueous emulsion of paraffin containing aluminium salts  
 50 g. glycerine

1000 g.

After drying and steaming for 5 minutes in the rapid-steaming apparatus, the product is transparentised and finished in the described way.

The result is a plastic white contrast pattern on a light blue ground.

I claim:

- 5 1. A process for producing patterns on a cotton textile comprising the steps of printing a pattern on the textile with a composition comprising an acid stable mineral pigment and an aqueous emulsion of an oleaginous substance, the oleaginous substance being the sole pigment binding agent present, drying the printed textile, and thereafter treating the printed textile with an acid transparentizing agent, whereby the non-printed portion of the textile is transparentized and the pigment is bonded to the printed portion thereof, and thereafter washing the textile to remove the unbound surplus of pigment.
- 10 2. A process for producing figured cotton textile goods comprising the steps of printing a pattern on the goods with a printing paste comprising an aqueous emulsion of an oleaginous substance, a thickening agent, and an acid stable mineral coloring substance, the oleaginous substance being the sole pigment binding agent present, drying the printed goods, and thereafter treating the goods with a transparentizing agent for the purpose of transparentizing the non-printed areas and bonding said coloring substance to the fibers defining the printed areas of the goods.
- 15 3. A process for producing a figured cotton textile which comprises the steps of printing a pattern on defined areas of the textile with a composition comprising an acid stable mineral pigment and an aqueous emulsion of paraffin, the paraffin being the sole pigment binding agent present, drying the printed textile, and treating the dried textile with an acid transparentizing agent.
- 20 4. A process for producing a figured cotton textile which comprises the steps of printing a pattern on defined areas of the textile with a composition comprising an acid stable mineral pigment and an aqueous emulsion of paraffin, the paraffin being the sole pigment binding agent present, drying the printed textile, steaming it wet, treating the dried textile with concentrated sulphuric acid, whereby the non-printed areas are transparentized and the pigment is bonded to the fibers in the printed areas, and thereafter washing the textile to remove the unbound surplus of pigment.
- 25 5. A process for producing a figured cotton textile which comprises the steps of printing a pattern on defined areas of the textile with a composition comprising an acid stable mineral pigment and an aqueous emulsion of paraffin, the paraffin being the sole pigment binding agent present, drying the printed textile, treating the dried textile with an acid transparentizing agent, and tensioning said textile during the said acid treatment.
- 30 6. A process for producing a figured cotton textile which comprises the steps of printing a pattern on defined areas of the textile with a composition comprising an acid stable mineral pigment and an aqueous emulsion of an oleaginous substance, the oleaginous substance being the sole pigment binding agent present, drying the printed textile, steaming it wet, treating the dried textile with concentrated sulphuric acid, whereby the non-printed areas are transparentized and the pigment is bonded to the fibers in the printed areas, and thereafter washing the textile to remove the unbound surplus of pigment.

7. A cotton textile product obtained by the process claimed in claim 1.

HEINZ GINZEL.

**REFERENCES CITED**

The following references are of record in the file of this patent:

**UNITED STATES PATENTS**

| Number    | Name   | Date         | Number     |
|-----------|--------|--------------|------------|
| 2,080,509 | Schoen | May 18, 1937 | 10 413,150 |

| Number    | Name             | Date          |
|-----------|------------------|---------------|
| 2,171,513 | Heberlein et al. | Aug. 29, 1939 |
| 2,174,534 | Shipp            | Oct. 3, 1939  |
| 2,202,200 | Haller et al.    | May 28, 1940  |
| 2,275,991 | Powers           | Mar. 10, 1942 |
| 2,298,147 | Miller           | Oct. 6, 1942  |

**FOREIGN PATENTS**

| Country       | Date          |
|---------------|---------------|
| Great Britain | July 12, 1934 |